

1

2,829,101

## SULFURIZED CUTTING OIL COMPOSITIONS

Jacobus Rinse, Bernardsville, N. J., assignor to Sulfo-Inc., Elizabeth, N. J., a corporation of New Jersey

No Drawing. Application January 19, 1954  
Serial No. 405,050

6 Claims. (Cl. 252—31)

This invention relates to sulfurized cutting oils and more specifically to such oils of improved properties in which the suspension of the finely divided sulfur is caused and maintained by the presence of a small amount of an ester of hydroxy stearic acid.

Cutting oils of the type here involved are described in the United States patent of Victor R. Abrams, No. 2,157,379, the sulfur being suspended in the cutting oil base by means of a hydrogenated castor oil wax which provides a free flowing gelatinous mass. Although these cutting oils serve their intended purpose quite well, they do not provide ideal performance, particularly in relation to sedimentation. In addition, the suspending agent is of limited availability. Other cutting oils used in industry are even more deficient as to this sedimentation quality.

An object of the present invention is to provide cutting oils having highly effective improved properties. Another object is to produce cutting oils which remain stable and homogeneous over long periods of time and which are capable of substantial dilution with mineral oil without loss, or appreciable loss, of stability.

The sulfurized cutting oils of the present invention are composed of a mineral oil base, finely divided sulfur and a suspending agent composed of an ester of any of the hydroxy stearic acids known to industry among which there may be mentioned the alpha- and beta-hydroxy, and the 10-, 11-, and 12-hydroxy stearic acids. These are esterified with a mono-, or a polyvalent alcohol preferably those of low and intermediate chain length as up to eight carbon atoms to provide a mono-ester. Specifically, there may be utilized esters from aliphatic alcohols as methyl, hexyl, and ethylene glycol; aromatic alcohols such as benzyl; and cyclic alcohols such as cyclohexanol.

These hydroxy fatty acids may be derived by any of the known processes, and can be satisfactorily prepared either by hydroxylating stearic acid or by separation from castor oil. The alcohol used must produce esters of the acids which are sufficiently soluble in mineral oil.

No change from known practices as to the nature of the oil base or of the sulfur components is required either as to quality or proportions. As to the oil, the usual mineral or petroleum oils are contemplated, as those having a viscosity of 100-300 seconds. As to the sulfur component, flowers of sulfur and other finely divided sulfurs of particle sizes known to be suitable in providing cutting oils, are contemplated. The sulfur content of the cutting oil will usually amount to from about 1 to 10%, but the oil can be diluted further by the addition of more of the mineral oil base.

The novel cutting oils of the present invention composed predominantly of the mineral oil base require only a small amount of the ester to produce and maintain the suspension of the sulfur. The proportion required in any particular formulation depends upon the viscosity of the oil, the proportion and particle size of

2

the sulfur, the suspending power of the particular ester used and the conditions of use intended for the cutting oil, and can be determined by test. The amount added, of course, should be large enough to effect the stable suspension without at the same time preventing the degree of free flow required of the cutting oil during the intended use. Usually a proportion amounting to about 2 to 10 percent gives desirable results.

The sulfurized cutting oils may be compounded without difficulty in any stirring or agitating device. The components may be added in any order but a procedure serving well involves first dispersing the ester in the mineral oil and then adding the finely divided sulfur as such or dispersed in a lighter or a heavier hydrocarbon oil.

Although the cutting oils of the invention serve well their intended purposes without any additions, it is realized that for specific reasons arising in their use throughout the industry it will be desirable to add other components, as lard oil or other animal oils; vegetable oils, as cotton seed oil, rosin or rosin oil; hydrogenated oils, turpentine, carbon tetrachloride, kerosene, sulphonated lard oil, soaps or even water or graphite.

### Example 1

To 95 parts of mineral oil (200 sec. visc.) there are added 5 parts of methyl 12-hydroxy stearate. The mixture is heated until a completely homogeneous mass is obtained. Thereupon, 15 parts of flowers of sulfur are mixed in and a paste is obtained which remains homogeneous during storage. When it is to be used as a cutting oil, it can be diluted with 100-200% of its weight with additional mineral oil.

### Example 2

To 6.25 parts of ethylene glycolate of 10-, 11- or 12-hydroxy stearic acid, there are added 250 parts of mineral oil (100 sec. visc.). The mixture is heated until a homogeneous mass is obtained. After the mass cools, 25 parts of sulfur are added and stirred in. The resulting suspension remains homogeneous for more than six weeks. It can be diluted with an equal weight of the same cutting mineral oil base and the sulfur will not settle out from the suspension formed even if stored for an additional six weeks.

### Example 3

Twelve and one-half parts of butylhydroxy stearate are dissolved by mixing in 250 parts of hot mineral oil (200 sec. visc.). After the mass cools, 25 parts of flowers of sulfur are added and stirred in. The resulting suspension remains stable for a period of more than six weeks and performs well as a cutting oil after dilution with two times up to as much as five times more mineral oil.

It should be understood that the present invention is not limited to the specific compounds or materials disclosed herein but that it extends to all equivalents which will occur to those skilled in the art upon consideration of the terms of the claims appended hereto.

I claim:

1. A sulfurized cutting oil comprising a mineral oil having the properties required for use in cutting oils containing finely divided sulfur suspended therein by the presence of a small amount of an ester of hydroxy stearic acid having up to eight carbon atoms in the esterifying radical.

2. A stable, free-flowing, sulfurized cutting oil comprising a cutting oil base composed of mineral oil, flowers of sulfur suspended therein and a suspending agent consisting of a mono-ester of hydroxy stearic acid

3  
in a quantity which stably suspends said sulfur particles while permitting free flow of the cutting oil during use.

3. A sulfurized cutting oil comprising a mineral oil having the properties required for use in cutting oils containing finely divided sulfur suspended therein by the presence of a small amount of a lower molecular alkyl ester of hydroxy stearic acid. 5

4. A sulfurized cutting oil comprising a mineral oil having the properties required for use in cutting oils 10 containing finely divided sulfur suspended therein by the presence of a small amount of the butyl ester of hydroxy stearic acid.

5. A sulfurized cutting oil comprising a mineral oil having the properties required for use in cutting oils 15 containing finely divided sulfur suspended therein by the presence of a small amount of the ethylene glycolate of hydroxy stearic acid.

6. A sulfurized cutting oil comprising a mineral oil having the properties required for use in cutting oils 20

4  
containing finely divided sulfur suspended therin by the presence of a small amount of the methyl ester of hydroxy stearic acid.

References Cited in the file of this patent

UNITED STATES PATENTS

1,913,300 Abrams ----- June 6, 1933  
2,157,379 Abrams ----- May 9, 1939

FOREIGN PATENTS

329,266 Great Britain ----- May 5, 1930

OTHER REFERENCES

"Synthetic Detergents," by McCutcheon, MacNair-Dorland Co., New York, N. Y., 1950, pages 46 and 47.

Gregory: "Uses and Application of Chemicals and Related Materials," Reinhold Publishing Corporation, New York, N. Y., 1939, vol. 1, page 322.